

# UNITED STATES PATENT OFFICE.

WILLIAM LOESCH, OF CHICAGO, ILLINOIS, ASSIGNOR OF FORTY ONE-HUNDREDTHS TO  
GEORGE B. STORER, OF CHICAGO, ILLINOIS.

## FUEL-BRIQUET COMPOSITION FOR IRON-ORE REDUCTION.

1,131,531.

Specification of Letters Patent.

Patented Mar. 9, 1915.

No Drawing.

Application filed April 14, 1913. Serial No. 761,126.

To all whom it may concern:

Be it known that I, WILLIAM LOESCH, a citizen of the United States residing at Chicago, in the county of Cook and State of Illinois, have invented certain new and useful Improvements in Fuel-Briquet Compositions for Iron-Ore Reduction Processes; and I do hereby declare the following to be a full, clear, and exact description of the invention, such as will enable others skilled in the art to which it appertains to make and use the same.

The invention relates to compositions for making fuel briquets suitable for use in reducing iron ore, and has for its object the provision of a briquet using the waste from coke furnaces and providing a briquet that will not disintegrate under the heat of combustion required in reducing iron ore and the provision of limestone that acts as a flux required in the process of reducing iron ore.

In making my improved briquet I take one hundred (100) parts by bulk of coke dust and screenings that are the waste product of coke ovens and add thereto from one (1) to two (2) parts by bulk of coal oil thoroughly mixing the coal oil with from five (5) to ten (10) parts, by bulk, of ground limestone, the limestone being reduced to a substantially No. 20 powder. I then take twenty-five (25) parts by bulk, of cement, either Portland or slag, and mix with the cement twenty-five (25) parts by bulk, of water forming a liquid solution which is afterward thoroughly incorporated with the coke dust and screenings, the coal oil and the ground limestone heretofore referred to.

The mixing of the ingredients can be accomplished by hand if desired but I prefer to use a concrete mixer of any preferred type in order to thoroughly mix the different ingredients to a plastic mass. The plastic composition heretofore described is then placed in molds of suitable size and shape and allowed to remain in said molds until the composition hardens, when the mold blocks are removed from the molds and thoroughly dried.

The blocks are used for fuel in the ordinary way and it has been found that the block retains its integrity under the heat of combustion and is not reduced to a powder except as the fuel products are consumed leaving the cement and limestone to pass off from the furnace in the shape of "slag" along with the other waste products of the iron ore in the course of reduction to the metallic state.

Having thus described my invention, what I claim is:

A plastic composition for forming fuel briquets for iron and ore reduction processes consisting of substantially one-hundred (100) parts of finely comminuted coke, from two (2) to five (5) parts of crude petroleum, from five (5) to ten (10) parts of ground limestone, twenty-five (25) parts of cement, and twenty-five (25) parts of water, said composition being mixed together and molded into briquets.

In testimony whereof I affix my signature in presence of two witnesses.

WILLIAM LOESCH.

Witnesses:

GEORGE B. STORER,  
JAS. A. FOLEY.